

## UNITED STATES PATENT OFFICE

JOHN A. GANN, OF MIDLAND, MICHIGAN, ASSIGNOR TO THE DOW CHEMICAL COMPANY, OF MIDLAND, MICHIGAN, A CORPORATION OF MICHIGAN

## PURIFYING LIGHT METAL

No Drawing.

Application filed October 4, 1928. Serial No. 310,440.

As is well known, crude magnesium, such as electrolytic cell metal, is often relatively impure, the impurities consisting largely of non-metallic ingredients, and where the metal to be used is remelted scrap magnesium metal and/or its alloys, it is equally important that steps be taken to eliminate foreign matter, if clean castings are to be secured either in the form of stock bars or finished articles. 5 One such method is described in my co-pending application Ser. No. 651,431, filed July 10, 1923, now Patent No. 1,754,788.

The object of the present invention is the provision of a further improved method for 15 eliminating such impurities either in the case of magnesium metal or of so-called light metal alloys in which magnesium is the predominant ingredient.

To the accomplishment of the foregoing and related ends the invention, then, consists of the steps hereinafter fully described and particularly pointed out in the claims, the following description setting forth but one of the various ways in which the principle of 25 the invention may be carried out.

The main step in my improved process consists in the washing or thorough intermixture of the metal or such alloy thereof while in molten condition with a suitable fluxing material. Several different fluxes have been described and used either in connection with the electrolytic production of magnesium or as a coating for the metal in molten state in order to protect the same against oxidation 30 which becomes excessive where the molten metal is exposed directly to the atmosphere. Anhydrous magnesium chloride, which is one of the materials employed in the electrolytic production of the metal, serves also when in 35 molten condition as a flux or protective coating but has too high a melting point when used alone so that sodium chloride is ordinarily added to lower such melting point. The flux thus composed of magnesium chloride 40 and sodium chloride is disclosed in U. S. Patent No. 1,377,374 and also in German Patent No. 122,312, the latter describing a flux consisting of equimolecular weights of magnesium chloride, sodium chloride and potassium chloride with the addition of a small 45

amount of calcium fluoride. U. S. Patent No. 1,476,192 discloses a flux consisting of magnesium and sodium chlorides in approximately equal proportions with a relatively small amount of barium chloride added to 55 raise the specific gravity of the flux slightly above that of the metal, either magnesium alone or an alloy thereof, with which it is to be used. A different type of flux is disclosed in U. S. Patents, Nos. 1,576,080 and 1,661,526, which describe the use of a small amount of flux to which is added various compounds so that it will be thick and pasty while the metal is being purified.

In the practice of my present improved 65 method of purification, any suitable flux may be employed in which the proportion of ingredients is such that the melting point of the mixture is lower than that of the metal or alloy and at the same time such flux mixture, when in molten state, is limpid and mobile, and has a surface tension such as to cause it to coat the exposed surface of the metal. Such flux, as for instance that mentioned in the said Patent No. 1,476,192, will 70 also preferably have a slightly higher specific gravity than the metal or alloy so that the latter will float in the relatively large bath of flux to be used, in other words, it is proportionately large when compared with the 75 volume of metal it floats and coats. When using a flux of this type I have found that in general the coefficient of expansion of the molten flux is greater than that of molten metal. Thus the higher the temperature of 80 the molten bath is raised, the more the flux will rise to form an increasingly thicker protective film on the upper surface of the metal. At sufficiently high temperature the ratio of 85 densities is even reversed, so that the metal floats the flux. This tendency results in the metal being increasingly better protected by the flux as the temperature of the molten metal is raised to the desired washing point.

A batch of the metal or alloy containing 90 impurities as aforesaid is melted down in a pot containing a sufficient quantity of such flux material to float and effectively coat the upper surface of the body of metal when in molten state. According to the preferred 95 100

procedure, the flux employed at this stage may in some cases be that resulting from a subsequent step in the purification treatment as will presently appear. As soon as the 5 metal is in proper fluid state, the flux of course being likewise fluid at the temperature involved, the metal is gently agitated or stirred with the flux so as to be thoroughly washed therewith without dispersion of the 10 metal therein. At the same time the temperature of the molten bath may be raised, e. g., to a point as high as 300° C. above the melting point of the metal, whereby the metal and flux are both made very limpid and mobile, and a more thorough washing and purification of the metal from non-metallic impurities can be accomplished. The limpid and mobile mixture is then allowed to stand 15 quietly to settle out the flux and impurities 20 while the metal is cooling back to the desired casting temperature. If the metal were relatively clean at the start of the process, this one purification will be all that is necessary to prepare the metal for casting. However, 25 if the metal were relatively dirty at the start, a still further purification step will sometimes be necessary. In such case, when the metal has cooled back to the desired temperature it is dipped or otherwise transferred 30 into another pot containing a fresh lot of substantially pure flux where it is again gently agitated or stirred in the fashion just described and allowed to stand. This retreatment with clean flux I find will remove substantially all of the remaining non-metallic 35 impurities from the magnesium or its alloy and the metal will be then in suitable condition for casting.

The purified body of metal, or at least the 40 major portion thereof, obtained as a result of the last step, is transferred at suitable temperature directly from the pot to the molds, leaving behind the flux with the impurities taken up thereby from such body of 45 metal. This flux is then used in repeating the first step wherein the crude metal with maximum content of impurities is melted down and agitated as hereinbefore set forth. None of the metal from the second step that 50 is left in the flux bath is of course lost since it is mingled with the raw metal added in repeating the first step.

In order to ladle the metal from one pot to the other, the thin film of the flux that overlies the surface of the molten mass of metal in the pot is broken and brushed to one side so as to uncover the clear metal and the ladle can then be filled and lifted before the film is re-established. However, where proper 55 precautions are taken, such re-establishment of the film will occur before any oxidation or other harmful effect is produced on the exposed metal and by careful manipulation the operator is at the same time able to avoid 60 taking up any of the flux in the ladle. It

will be understood, of course, that the method of purification in hand is not limited to any such particular method of transferring the metal. It will also be understood that I may increase the number of successive operations wherein progressively cleaner flux is employed instead of operating simply in one or two stages as described. 70

While the molten metal and flux may be continually agitated or stirred while being heated to a temperature as high as 300° C. above its melting point, I have found that it is generally sufficient to gently and thoroughly agitate or wash the metal with the flux at approximately the highest temperature attained. At this point the metal and flux are both very limpid and mobile, and a thorough washing of the former is easily attained. 75

The term "light metal" as used herein will be understood to designate either magnesium by itself or alloys of the character hereinbefore described wherein magnesium is the predominant constituent. Similarly, the term "scrap" will be understood as designating any form of such light metal, whether shavings, turnings, chippings, fragments of castings, or the like, with which objectionable foreign matter is in any way intermixed or included. 80

Other modes of applying the principle of my invention may be employed instead of the one explained, change being made as regards the method herein disclosed, provided the step or steps stated by any of the following claims or the equivalent of such stated 100 means be employed.

I therefore particularly point out and distinctly claim as my invention:—

1. The method of purifying magnesium and alloys thereof which comprises melting the metal in a proportionately large bath of a mobile molten flux, temporarily subjecting the molten mixture of metal and flux to a temperature of about 100° to 300° C. above the melting point of the metal, whereby to increase the fluidity of such flux, agitating the molten metal with the flux whereby non-metallic impurities are removed from the metal by the washing action of the flux, allowing the mixture to stand quietly to segregate the flux and the metal, while cooling to a casting temperature, and separating the metal from the flux. 105

2. The method of purifying magnesium and alloys thereof which comprises melting the metal in a proportionately large bath of a mobile molten flux, temporarily subjecting the molten mixture of metal and flux to a temperature of about 100° to 300° C. above the melting point of the metal, whereby to increase the fluidity of such flux, agitating the molten metal with the flux whereby non-metallic impurities are removed from the metal by the washing action of the flux, allowing the mixture to stand quietly to seg- 110 115 120 125 130

regate the flux and the metal, while cooling to a casting temperature, separating the metal from the flux, and repeating the foregoing treatment with another body of flux.

5. The method of purifying magnesium and alloys thereof which comprises melting the metal in a proportionately large bath of a mobile molten flux containing magnesium chloride, temporarily subjecting the molten mixture of metal and flux to a temperature of from 100° to 300° C. above the melting point of the metal, agitating the molten metal with the flux, allowing the mixture to stand quietly to segregate the flux and the metal while 10 cooling to a casting temperature and separating the metal from the flux.

4. The method of purifying magnesium and alloys thereof which comprises melting the metal in a proportionately large bath of a mobile molten flux containing magnesium chloride, temporarily subjecting the molten mixture of metal and flux to a temperature of from 100° to 300° C. above the melting point of the metal, agitating the molten metal with the flux, allowing the mixture to stand quietly to segregate the flux and the metal while 20 cooling to a casting temperature, separating the metal from the flux, and repeating the foregoing treatment with another body of flux.

Signed by me this 2nd day of October, 1928.

JOHN A. GANN.